

## UNITED STATES PATENT OFFICE

2,358,788

PRODUCTION OF SILICON STEEL OF  
UNIFORMLY LOW CORE LOSS

Victor W. Carpenter, Franklin, and John M. Jackson, Middletown, Ohio, and Jack E. Lucas, Butler, Pa., assignors to The American Rolling Mill Company, Middletown, Ohio, a corporation of Ohio

No Drawing. Application August 3, 1940,  
Serial No. 351,126

9 Claims. (Cl. 148—12)

Our invention relates to the production of silicon steel for electric uses and has for its principal object the attainment of uniformly low core loss in low carbon silicon steels without significant increase in cost.

In the copending application of Victor W. Carpenter entitled Method of producing silicon steel sheet or strip, Ser. No. 60,347, filed January 22, 1936, now Patent No. 2,236,519, issued April 1, 1941, there are set forth processes for the production of silicon steel characterized broadly by a decarburizing treatment between the hot rolling and cold rolling stages, which treatment is a box annealing of the material in the presence of the hot mill scale. This treatment is inexpensive and is effective in reducing the carbon content to .015% or lower irrespective of the starting carbon in commercial silicon steels. In material of such low carbon content a final box annealing can be dispensed with, since the grains grow so rapidly that the development of the desired magnetic properties can be achieved in a commercial continuous anneal of the single strand type. The treatment has come into use for many grades of silicon steel manufactured by us.

Most cold rolled silicon steel is sold on a core loss guarantee. Each commercial grade is made from a selected silicon grade of bar stock, by a series of operations appropriate to the particular result desired. In spite of the close adherence to standardized practices it has been found that variables in the processing or analysis which are not easily controlled may influence the final product to such an extent that certain batches of material may not meet the core loss guarantee. After examination of such batches of material over a long period of time, we have found, when other factors have been calculated to a comparable basis, that the difficulty accompanies too small a grain size in the finished product. We therefore came to the conclusion that greater uniformity in achieving the lower core losses which we obtain, implied a variation in procedures to obtain a larger grain size on the average;—or, putting it another way, greater consistency in core loss results would follow greater consistency in the production of a large grain size in the finished product.

It has been known that very large grains may be obtained in cold rolled silicon steel by "strain rolling." This is essentially a finishing operation involving annealing the cold rolled sheet or strip when it is within a few thousandths of an inch of final gauge, cold rolling it to gauge, and

then again annealing it. Strain rolling is expensive, introducing as it does an extra anneal and a cold rolling of only a few thousandths of an inch, which requires a very accurate control. This expense is justified only on the higher grades of silicon steel.

It was our purpose to evolve a treatment which would produce a uniformly larger grain size than was possible without "strain rolling" but which would be available for substantially all silicon steel grades because of relatively slight cost. The known operation of strain rolling was therefore not seen as available for our purpose. We have determined, however, that the grain size of the hot-rolled material (or hot-rolled material which has been annealed) will determine the ultimate grain size in the cold rolled and annealed product. The larger the original grain size, the larger will be the final grain size within certain limits. Thus, if the original hot-rolled thin bar could be made to have a larger grain structure, uniformly, we believed we would secure the desired improvement and uniformity in the final product. Experience has shown that this is the case.

There are several methods by which a larger grain structure may be secured in the thin bar. A higher annealing temperature following the hot rolling will give larger grains. Also, if the hot rolling is finished at such a temperature as to leave considerable strain in the thin bar, grain growth will occur during the subsequent box anneal. Conversely, it is possible to finish the hot rolling at such a high temperature that large grains are present in the bar as delivered from the hot mill.

All of these factors give a measure of control and are useful alone or in combination with each other or with the more definite factor next to be discussed. We find that good results can be more certainly attained and controlled by introducing strain into the hot-rolled bar after the hot rolling so that large grains will grow during the box anneal. There are various methods of accomplishing this purpose; but they all involve a working of the piece. The piece may be given one or more passes through a scale breaker, and this will be found to introduce sufficient strain to produce useful grain growth or the piece may be strained after the hot rolling by passing it through an ordinary cold mill. Both of these procedures can be carried on so as not to remove the hot mill scale from the hot-rolled part whereby the efficacy of the following box anneal as a decarburizing treatment is not impaired. The

cold rolling where adopted (and where the anneal is to be decarburizing anneal) is a cold rolling in the presence of the hot mill scale.

In an exemplary practice employing a scale breaker, we gave the thin bar two passes through the apparatus: We did this in the particular instance so that the first ten feet of the bar, which were utilized in threading the machine and which therefore did not receive the straining on the first pass, would be strained on the second pass. The scale breaker treatment is somewhat less expensive than the cold rolling; but the use of the mill for straining results in more uniform grain size.

We have examined microscopically materials which have been strained by being passed through a scale breaker after the box anneal which follows. These materials were found to have large grains on each surface, which extended toward the midthickness of the bar about one-fourth of the way through the bar. Thus the box annealed bars made in this way contained large grains which comprised approximately one-half of the total thickness of the bar. The grains at the midthickness were of the size which would be obtained in the box annealed bars without the straining. Nevertheless, the amount of material characterized by large grains in the box annealed product was found sufficient to produce the desired large grains after the complete process of making the silicon steel sheets had been gone through. When the pieces strained by cold rolling are examined, the grain growth due to straining is found to be much more general and uniform throughout the thickness of the piece.

As an outline of a general process which we heretofore carried out, we hot-roll silicon steel to a gauge say from .06 to .10 inch. We then box anneal the strip in the presence of the mill scale whereby to decarburize it. Thereafter we pickle the strip, cold roll it to the final gauge, and open anneal it. This process as modified in accordance with the present invention may be summarized as follows: Hot roll to from .06 to .10 inch, introduce a critical amount of strain into the bar, box anneal, pickle, cold roll to final gauge, and open anneal. It will be noted that we have not added significantly to the cost of the process; but the uniformity of results and general improvement in results which we secure is marked and valuable.

As to the various factors affecting grain size of the hot-rolled material, all of these have a certain importance and combinations of them are contemplated by our invention. Even where chief reliance is placed upon a definite working of the metal after it has cooled from the hot rolling temperature, the other factors of control may be utilized. Moreover, the various conditions should preferably be known. For each box annealing temperature and grade of material there is a theoretical critical amount of strain necessary to cause large grains to grow, which relationship is described in numerous places in the technical literature. This amount of strain varies with the factors which we have outlined; but in the light of our teachings it is within the skill of the worker in the art to select a proper amount of working and a proper annealing temperature in view of the other factors for the desired grain growth. For example, using a medium silicon of around 2% we have found that around 7 to 8% reduction will result in a

satisfactorily large grain size after a subsequent box anneal at 1400° F.

Our process is applicable to any of the hot-rolled gauges of silicon steel that are now being used. The essential limitation upon the hot-rolled gauge is that of the power and capacity of the hot mills. Moreover, our invention applies to hot-rolled thin bars or the like of any silicon content, which are usable to produce cold rolled strip. The silicon content of the material also is a factor which has some bearing upon the amount of strain necessary to produce large grains.

The application of our new process results in an enlargement in grain size over the same process with the new step omitted. It is not to be understood that it will produce grains quite as large as those resulting from the use of the more expensive "strain rolling" process which has been described. The improvement resulting from the use of our process, however, is of such an order as to significantly enhance the magnetic properties of the material.

Modifications may be made in our invention without departing from the spirit of it. Having thus described our invention, what we claim as new and desire to secure by Letters Patent is:

1. A process of producing silicon steel sheet or strip characterized by enlarged grain size, which comprises hot-rolling silicon steel to an intermediate gauge, introducing a critical strain by cold work into the hot-rolled material, box annealing it, thereafter cold rolling it to final gauge with a large percentage reduction substantially in excess of percentage reductions for critically straining it, and finally heat treating the silicon steel, to develop its magnetic properties and a large grain size.

2. A process as claimed in claim 1 wherein the introduction of the strain is accomplished by passing the hot-rolled material through a scale breaker.

3. The process as claimed in claim 1 wherein the strain is introduced into the hot-rolled material by giving it a pass through a cold mill prior to the initial annealing.

4. The process as claimed in claim 1 wherein the strain is introduced into the hot-rolled material by giving it a pass through a cold mill prior to the initial annealing, the hot-rolled material as passed through said cold mill bearing the hot mill scale on its surfaces.

5. A process of producing low carbon silicon steel sheet or strip which comprises hot-rolling silicon steel to an intermediate gauge, cooling the silicon steel, introducing a critical strain by cold work into the silicon steel, and thereafter box annealing the silicon steel without removal of the hot mill scale, thereafter cold rolling the silicon steel to final sheet gauge by producing therein a cold rolling reduction substantially in excess of percentage reductions for critically straining it, and heat treating it to develop its magnetic properties and a large grain size.

6. A process of producing low carbon silicon steel sheet or strip which comprises producing hot-rolled silicon steel of an intermediate gauge characterized by critical strain productive of a large grain size upon annealing, annealing said silicon steel in the presence of the scale resulting from hot-rolling, whereby to decarburize it, pickling the silicon steel, cold rolling it to final sheet gauge by producing therein a cold rolling reduction substantially in excess of percentage reductions for critically straining it, and finally an-

nealing the silicon steel to develop its magnetic properties and a large grain size.

7. A process of producing silicon steel sheet or strip which comprises hot-rolling silicon steel to a gauge of substantially between .06 and .10 inches, introducing critical strain into the hot-rolled silicon steel, box annealing it, pickling it, cold rolling it to sheet gauge with percentages of cold rolling reduction substantially in excess of percentages for critically straining it, and thereafter open annealing it to develop its magnetic properties and a large grain size.

8. The process as claimed in claim 7 in which the box anneal is carried on in the presence of the hot mill scale so as to decarburize the silicon steel as well as cause grain growth therein.

9. A process of producing low carbon silicon steel sheet or strip of enlarged grain size, which comprises producing hot rolled silicon steel of

5 an intermediate gauge of approximately from .06 to .10 inch, cooling the hot rolled silicon steel to cold rolling temperatures, cold rolling it without removing the hot mill scale from its surfaces, and with only sufficient elongation to produce a critical strain in the silicon steel, thereafter box annealing the silicon steel still in the presence of the hot mill scale, whereby to decarburize it by reducing the carbon therein from a higher value to approximately a maximum of .015%, pickling the silicon steel, cold rolling it to final sheet gauge by producing therein a cold rolling reduction of at least around 50%, and finally annealing the silicon steel to develop its magnetic properties and a large grain size.

VICTOR W. CARPENTER.  
JOHN M. JACKSON.  
JACK E. LUCAS.